

Patented Jan. 3, 1928.

1,655,097

# UNITED STATES PATENT OFFICE.

ERNEST K. GLADDING, OF BUFFALO, NEW YORK, AND THOMAS E. SHARPE, OF OLD HICKORY, TENNESSEE, ASSIGNEES TO DU PONT RAYON COMPANY, INCORPORATED, OF BUFFALO, NEW YORK, A CORPORATION OF DELAWARE.

## TREATMENT OF RAYON.

No Drawing.

Application filed March 27, 1926. Serial No. 97,981.

This invention relates to the manufacture of artificial fibers, such as rayon. It has been found that the finished product shows discoloration in the form of greenish spots or streaks. The reason for this discoloration was unknown for a long time, but we have discovered that it is caused by the presence of certain metal, such as copper, in the water which is used to wash the fibers.

10 These metals may not be present in the water in large percentages but still the aggregate may be large, because of the fact that a very great quantity of water is employed. For example, in the manufacture of rayon

15 by the method employing glass bobbins between 1,500 and 2,000 pounds of water are used in washing one pound of rayon. It is not unusual to find 0.05 parts of copper per 1,000,000 parts of water, and this proportion, although small, is equivalent to 0.04

20 grams of copper for the 2,000 pounds of water which may be used in washing one pound of rayon. The above figures are given as showing that the total amount of 25 copper which may come in contact with the rayon during its manufacture may be large enough to do considerable damage. The discoloration referred to above not only detracts from the appearance of the product

30 but also materially weakens it.

It is, therefore, the object of our invention to provide a method of treating artificial fibers which shall remove the above contamination. This object we achieve by treating 35 the fibers after they have been washed in the water, which water is apt to contain the copper, with a solution of a metal cyanide, such as sodium cyanide or potassium cyanide. A water soluble cyanide is preferable.

40 A still further object of our invention is to provide a method as set forth above and which shall be safe in operation for the persons practicing the same. The metal cyanide which we preferably employ is sodium cyanide, and this substance reacts with any traces of acid which at this stage may be 45 present in the rayon to produce hydrogen cyanide or prussic acid which is very volatile and the vapors of which are highly 50 poisonous. We, therefore, incorporate in the bath or in the substance with which we treat the fibers an alkali which will pre-

vent the formation of a volatile poisonous compound.

55 For the purpose of illustration we shall describe our invention as practiced in the manufacture of rayon, although it is not limited thereto. The rayon may be treated with a metal cyanide in any suitable manner. Rayon, as it comes from the wash, may be 60 in the form of cakes or skeins. We will first describe a method of treatment of the cakes.

A bath is prepared containing sodium cyanide of a concentration of about 0.05% to about 0.2% and ammonium hydroxide of a concentration from about 0.05% to about 0.1%. In actual practice we have found that the concentrations of the above reagents may conveniently be made 0.2% and 0.1% respectively. The temperature of the bath is preferably maintained at about 40° centigrade. The cakes of rayon are moved through the bath or subjected to the action thereof by any suitable mechanism, for example, by a conveyor which may be arranged to carry or roll the cakes through the bath. The major part of the contamination occurs on the exterior of the cakes, and, therefore, it is unnecessary to subject the cakes to the action of the cyanide for an extensive period. We have found that one minute will normally suffice with the above concentrations. In this connection care must be exercised to prevent too long a treatment with the cyanide, which would result in a penetration 75 thereof into the cakes and which would then require a longer period of washing to remove the cyanide.

80 After passing through the cyanide bath, the cakes of rayon are then immersed in or subjected to a bath of warm water at a temperature approximating that of the cyanide bath. This water should be circulating, preferably, so as to insure a continual supply 85 of fresh water and thorough removal of the cyanide. We have found that a period of one minute is sufficient for the washing with water.

90 The temperatures which we have indicated above as desirable for both the cyanide and water baths are employed in order to hasten the rate of the chemical reactions involved and also the rate of removal of the cyanide 95 by the subsequent water washing.

100 The effectiveness of the above described

method may be seen from the following example. A bobbin of rayon was moistened with a dilute solution of copper sulfate and then exposed to the air of the spinning room, which air was contaminated with hydrogen sulfide. After about an hour the entire cake was found to be covered with a very black discoloration because of the formation of copper sulfide. The cake was then placed in a bath of dilute potassium cyanide, and after several minutes it was found that the black discoloration had entirely disappeared. This was because of the formation of a soluble compound of copper with the cyanide. It is well-known that copper salts in a solution containing an excess of potassium cyanide cannot be precipitated by hydrogen sulfide. This is because of the fact that there is formed the compound  $KCu(CN)_2$ , which ionizes almost completely as follows:



Copper thus being present as a part of the complex ion  $Cu(CN)_2^-$ , is not precipitated by hydrogen sulfide as would be the case with copper present in the form of copper ions.

Similarly, therefore, when the rayon upon the surface of which may be found a contamination in the form of a copper salt or copper in another form is treated with a metallic cyanide, much the same result probably follows, although the precise chemical reaction is unknown, because of the uncertainty as to the form in which the copper is originally present. It may occur in the water in the form of a soluble salt but more probably in a colloidal state, that is, in the form of insoluble particles in a very fine state of sub-division. However, regardless of the form in which the copper occurs, the above treatment effectually removes it.

The ammonium hydroxide employed in the cyanide bath is for the purpose of preventing the formation of hydrogen cyanide or prussic acid as stated above by reaction of the cyanide with any residual acid on the rayon. It is well-known that prussic acid is a very volatile compound and that its vapors are highly poisonous. It is, therefore, essential to prevent the escape thereof because of the consequent health hazard to the operators. The use of the ammonium hydroxide is an example of a method of maintaining a bath slightly alkaline, in order to immediately neutralize any residual acid which might be present in or on the cakes of rayon. Thus the formation of prussic acid is effectually prevented.

When the treatment with cyanide is to be applied to the rayon in the form of skeins, this may conveniently be done during desulfuring. Rayon in the form of skeins is usually desulfured and bleached by passing it under a series of showers of solutions of caustic soda and sodium hypo-chlorite re-

spectively. To the caustic soda solution may be added a quantity of sodium cyanide to effect a concentration of 0.025% to 0.1%. In this treatment the ammonium hydroxide is omitted, because the caustic soda furnishes the necessary alkali to prevent the formation of prussic acid.

While we have discussed contaminations caused by copper, it is to be understood that our invention is not limited to the removal of such contaminations alone, but is equally applicable to the removal of contaminations resulting from other metals. Throughout the claims we shall employ the term "metal" to cover all forms in which may be found the metallic substance which causes the contamination.

We claim:

1. The method of removing a metal contamination from artificial fibers which consists in treating the fibers with a metal cyanide. 85
2. The method of removing a metal contamination from artificial fibers which consists in treating the fibers with a water soluble metal cyanide. 90
3. The method of removing a metal contamination from artificial fibers which consists in treating the fibers with sodium cyanide. 95
4. The method of removing a metal contamination from artificial fibers which consists in treating the fibers with a warm solution of metal cyanide. 100
5. The method of removing a metal contamination from artificial fibers which consists in treating the fibers with a warm solution of a water soluble metal cyanide. 105
6. The method of removing a metal contamination from artificial fibers which consists in treating the fibers with a warm solution of sodium cyanide. 110
7. The method of removing a metal contamination from artificial fibers which consists in treating the fibers with a metal cyanide and an alkali. 115
8. The method of removing a metal contamination from artificial fibers which consists in treating the fibers with a water soluble metal cyanide and an alkali. 120
9. The method of removing a metal contamination from artificial fibers which consists in treating the fibers with sodium cyanide and an alkali. 125
10. The method of removing a metal contamination from artificial fibers which consists in washing the fibers with a solution containing sodium cyanide and ammonium hydroxide. 130
11. The method of removing a metal contamination from artificial fibers which consists in washing the fibers with a solution containing sodium cyanide and ammonium hydroxide and then washing the fibers with water. 135

12. The method of removing a metal contamination from artificial fibers which consists in treating the fibers with a desulfuring solution to which is added a metal cyanide. solution to which is added a water soluble metal cyanide. In testimony whereof, we have affixed our 10 signatures to this specification.
- 5 13. The method of removing a metal contamination from artificial fibers which consists in treating the fibers with a desulfuring

ERNEST K. GLADDING.  
THOMAS E. SHARPE.